

## UNITED STATES PATENT OFFICE

1,940,678

## PROCESS OF TREATING ALLOYS

Albert E. Fisher and Malvin A. Baernstein,  
St. Louis, Mo., assignors to National Pigments  
and Chemical Company, St. Louis, Mo., a cor-  
poration of Missouri

No Drawing. Application June 4, 1931  
Serial No. 542,096

8 Claims. (Cl. 75—1)

This invention relates generally to alloying of metals, and particularly to a process of forming alloys in which a material is added to the mix for removing the impurities and preventing segregation of the constituent elements.

In the processes of alloying metals which have been heretofore practiced, it has been necessary in practically every instance to employ some material as a so-called flux. The function of the various fluxes which have been employed has been to increase the fluidity of the alloy by lowering to some extent the temperature of fusion of the mixture. When the temperature of fusion is lowered by the addition of such a flux, it is apparent that the fluidity of the mix at a certain temperature will be substantially increased, and with the fluidity thus increased the tendency of the various constituent elements to segregate one from the other is substantially decreased. With the fluxes which have been heretofore employed, however, it has been found that they had a deleterious effect upon the furnaces or ladles in which the alloy is made. The various fluxes which have been heretofore employed have been as a general rule extremely basic in character and accordingly have an unusual effect upon the walls of the furnace or ladles as the case may be.

Among the objects of this invention is to provide a suitable fluxing agent for use in the alloying of metals which will not possess the disadvantages of the fluxes heretofore known in corroding or attacking the furnace or ladle in which the alloy is compounded.

In the processes which have been heretofore employed in the making of alloys, it has been impossible to prevent contamination of the alloy by foreign materials, such as are known as inclusions. For instance, in the various brasses some of the more common inclusions are silicon, aluminum and iron, and it has heretofore been impossible to remove these elements from any alloy in which they exist as impurities or inclusions. Many other impurities are also prevalent in the various alloys, such as for instance, sulphur and phosphorus which in many instances have an extremely deleterious effect upon the ultimate product and which may be present either in their combined or free form. It is among the objects of this invention, therefore, to provide a material which may be added to an alloy mix and which will be effective to remove the various impurities or inclusions as well as expelling the occluded gases.

An object of this invention is to provide a process of alloying metals which secures improved results.

Another object is to provide a fluxing agent for use in the alloying of metals.

A further object is to provide a purifying agent for use in the alloying of metals.

A more specific object is to provide a fluxing and purifying agent for use in the alloying of metals which will be effective to prevent segregation and expel the various inclusions as well as to increase the homogeneity of the ultimate product.

Another object of this invention is to provide a material for use in the making of alloys which is adapted to expel various undesired elements therefrom.

Other objects will become apparent to those skilled in the art when the following description is read:

In accordance with this invention a material may be added to the mix of molten alloy while in the furnace or ladle in which it was compounded, which acts both as a fluxing medium and purifier or cleanser. As an illustrative embodiment of this invention the material employed may be one known as tri-barium aluminate,

(3BaO·Al<sub>2</sub>O<sub>3</sub>),

80

which may be made in accordance with any suitable well known process. It is to be distinctly understood, however, that the invention is not limited to the use of the specific material mentioned.

In alloying the various metals for making brass, it is usually necessary to employ some fluxing medium for lowering the temperature of plasticity thereof, or increasing the fluidity of the mix at a certain temperature. In accordance with the present invention a material containing the oxides of barium and aluminum may be employed as such a flux and it has been found that such a material acts not only as a fluxing agent, but also as a purifier and cleanser. The reason for the purifying and cleansing action is to an extent at least from a theoretical standpoint, uncertain and it is, therefore, to be distinctly understood that the invention is not limited by any theoretical discussion or reasoning which may be given for the purpose of illustration herein.

When the compound, tri-barium aluminate, is added to the mass of molten metal the reaction which takes place is apparently due, in the first place, principally to the presence of barium. The barium apparently has a great affinity for the various inclusions or impurities such as sulphur, phosphorus and antimony, which are usually present in an alloy mix, such as for instance brass.

105

100

105

110

Moreover, in brass alloy, there is often present a small quantity of iron and silicon, as well as aluminum, and it is apparent that the compound, tri-barium aluminate, tends to throw off each of these various impurities, whether they exist in their combined or free forms. The action which apparently takes place upon the addition of the tri-barium aluminate to the molten alloy is apparently one of flocculation or coagulation, the tri-barium aluminate apparently tending to draw the various impurities out of solution and thus to increase the particle size thereof, by drawing together a great number of smaller particles into a single particle, or else by going into chemical combination with the various impurities. At the same time the material has a fluxing action upon the alloy, tending to increase the fluidity thereof at the existing temperature. In view of these two features the action which probably takes place upon the addition of the tri-barium aluminate to the alloy is simply one of decreasing the resistance to the movement of the included particles, and thus accelerating the movement thereof toward the surface where they may be oxidized and will remain as a scum or slag which may be readily removed in any suitable manner. It is possible that some oxidation of the various inclusions may take place before reaching the surface due to the presence of oxygen in the tri-barium aluminate. The action of the alumina in the material is difficult to determine, but it is evident that more beneficial results are obtained when the alumina is present than when barium oxide is used alone.

In the treatment of alloys with tri-barium aluminate as above described, the tendency of various constituent elements to segregate is substantially reduced. The reason for this is probably the great increase in the fluidity which is given the mix upon the addition of the tri-barium aluminate, it being recognized the greater the fluidity of the mass, the less the tendency for segregation. Perhaps the same reason may be given for the fact that in alloys which have been so treated there is an absence of occluded gases. With the fluidity of the mass so greatly increased, it is apparent that the resistance to the movement of gas bubbles toward the surface is substantially decreased so that the bubbles of occluded gases may readily move toward the surface and there be released.

Such a material as tri-barium aluminate shows a particular tendency for extracting antimony, sulphur and phosphorus from any alloy whether it be brass, a lead and tin alloy, an alloy of aluminum, a so-called base alloy or any other of the various alloys in which the antimony, sulphur and phosphorus are recognized as impurities. Moreover, the tri-barium aluminate has no corrosive effects upon the walls of the furnace or ladle and in fact acts as a cleanser therefor.

The various constituent elements of the fluxing and purifying material may, however, be deposited in the alloys in other compounds than that just discussed. For instance, a compound known as sodium barium aluminate and having a formula,  $(3\text{BaO}\cdot\text{Al}_2\text{O}_3)$  ( $\text{Na}_2\text{O}\cdot\text{Al}_2\text{O}_3$ ), which may be and preferably is made in accordance with the process disclosed in the copending application of Elbert E. Fisher, Serial No. 537,201, filed May 13, 1931 may be used, but it is to be distinctly understood that the invention is not limited to the specific materials which have been discussed, nor is it limited to such materials

as are made by the process described in the aforementioned application. Such a material as sodium barium aluminate contains all the constituents of tri-barium aluminate hereinbefore discussed and in addition thereto contains a substantial portion of sodium oxide. Under some circumstances it has been found that the presence of sodium is extremely beneficial, while under other circumstances the sodium content is of little or no importance. In general it is believed that the action of the sodium barium aluminate upon an alloy is in most respects the same as the action of the tri-barium aluminate although as above stated under some circumstances it has been found that the presence of sodium improves the action of the material both as a fluxing agent and a purifier. The reason for this improvement is, however, from a theoretical standpoint unexplainable.

It is apparent that when such a material as tri-barium aluminate, or sodium barium aluminate is employed as a fluxing and purifying agent in the alloying of metals, the occluded gases may readily move thru the molten mass and be expelled at the surface, and the various solid particles of inclusions may also readily move toward the surface where some will be to some extent oxidized and all the various impurities or inclusions will be held upon the surface of the alloy as a scum or slag. The scum or slag may be raked or scraped from the surface of the alloy by any suitable means. At the same time the fluidity of the alloy is so increased that the tendency of the constituent elements to segregate one from the other is substantially overcome and a homogeneous solution is thus maintained so that the ultimate product is not only free from occluded gases and impurities, but is extremely homogeneous.

It is to be understood that the expressions "oxides of sodium barium and alumina", "compound of barium sodium and alumina", and "sodium barium aluminate" are used herein and in the appended claims in their illustrative and not in their limitative senses. Where these expressions occur in the claims it is to be understood that those claims shall be construed of such scope as to cover equivalent materials.

From the foregoing description it is apparent that many modifications of this invention and the material employed as a fluxing and purifying medium will occur to those skilled in the art which will not depart from the spirit of this invention. It is to be distinctly understood, therefore, that the invention is not limited to the specific details which have been described and that such modifications thereof or the use of the process in the treatment of other alloys than those mentioned in the foregoing description, which do not depart from the spirit of this invention, and although not specifically described herein, are contemplated by and within the scope of the appended claims.

Having thus described the invention, what is claimed is:

1. In the art of alloying metals, the process comprising, adding to the mix a material containing tribarium aluminate.
2. In the art of alloying metals, the process comprising, adding to the mix a material containing tribarium aluminate and an oxy-sodium compound.
3. In the art of alloying metals, the process comprising, adding to the mix a material con-

- taining the oxides of barium, sodium and aluminum.
4. A purifying and fluxing agent for alloys comprising tribarium aluminate.
5. A purifying and fluxing agent for alloys comprising the oxides of barium, sodium and aluminum.
6. A purifying and fluxing agent for alloys comprising sodium barium aluminate.
7. In the art of alloying metals, the process comprising, adding to the mix a material containing sodium barium aluminate.
8. A purifying and fluxing agent for alloys, comprising, tribarium aluminate and an oxy- 80 sodium compound.
- ELBERT E. FISHER.  
MALVIN A. BAERNSTEIN.
- 10
- 15
- 20
- 25
- 30
- 35
- 40
- 45
- 50
- 55
- 60
- 65
- 70
- 75
- 85
- 90
- 95
- 100
- 105
- 110
- 115
- 120
- 125
- 130
- 135
- 140
- 145
- 150